

## UNITED STATES PATENT OFFICE.

ARMAND DE WAELE, OF LONDON, ENGLAND, ASSIGNOR TO D. GESTETNER, LIMITED, OF LONDON, ENGLAND.

## DUPLICATING.

No Drawing. Application filed June 15, 1923, Serial No. 645,707, and in Great Britain April 12, 1923.

This invention relates to duplicating manuscript and typewritten documents, drawings and the like by the employment of stencil sheets of the kind in which the 5 stencil layer is a disperse system comprising a gelatinized organic colloid deposited from an aqueous medium, that is, an organic colloid deposited from an aqueous medium in the form of a coherent gel and a 10 main tempering agent which does not form a true solution in the components of the disperse system, the main tempering agent being, for instance, an oily-waxy or waxy body, and which do not need moistening or 15 softening prior to cutting the stencil by means of a typewriter or style.

Stencil sheets of the kind in question having a stencil layer of the character indicated formed from gelatinizing organic 20 colloids which are peptized or dispersed in organic solvents and also others in which colloids, for instance gelatine, which are peptized or dispersed in an aqueous medium are present, although organic solvents have 25 in this case been used in forming the coating composition, are known. The employment of organic solvents is, however, open to objection on account of expense and, further, stencil sheets of the kind specified 30 formed from a gelatinizing organic colloid dispersible in an aqueous medium as hitherto produced have been found to be unsatisfactory.

The object of the present invention is to 35 provide improvements in connection with stencil sheets of the kind specified.

According to the present invention the main tempering agent is present in the composition, of which the stencil layer is constituted, prior to the gelation thereof, in 40 that degree of dispersion which is regarded as characteristic of the colloid state.

Thus, according to the invention, the composition may comprise a gelatinizing organic colloid dispersible in an aqueous medium and a tempering agent of the class described below which prior to the gelation of the composition is dispersed to the degree specified.

50 My investigations appear to show that the main tempering agent will be present in the composition after gelation in substantially the same degree of dispersion but that such is the case I have not yet been able to show

definitely. However, it would appear to be 55 characteristic of the gelated compositions constituting the stencil layer in accordance with the present invention, that the tempering agent is highly dispersed therein and most probably dispersed to the degree considered to be characteristic of the colloid state. This high degree of dispersion I have found to be necessary for securing a 60 highly sensitive stencil layer and at the same time a durable stencil.

65 In this connection it may be remarked that the tempering agents present in certain compositions constituting known stencil layers may be dispersed in the material after gelation to the degree considered to be 70 characteristic of the colloid state, but if this is in fact the case they have been present in the composition prior to gelation in the form of true or molecular solutions usually in the medium used for securing the 75 dispersion of the gelatinizing colloid.

The invention is not confined to the employment of particular organic colloids which will gelatinize but it may be remarked that organic colloids such as the 80 protein colloids, which peptize in aqueous media, may, in accordance with the invention, be employed in association with oily-waxy bodies or with waxy bodies and if necessary with an agent adapted to secure 85 the dispersion of the latter to the degree above indicated.

The invention consists more particularly in a stencil sheet having a stencil layer of the character specified broadly in the 90 above preceding paragraph, in which the oily-waxy bodies or waxy bodies present are soft or even liquid at the ordinary temperature of the air.

The invention also extends to the process 95 of forming stencil sheets which comprises applying to a porous support, for instance yoshino paper, an emulsion from which volatile organic solvents are absent, comprising a gelatinizing organic colloid dispersed in an aqueous medium, an oily-waxy body or waxy body and, if necessary, an agent adapted to secure the emulsification 100 of the latter in the organic colloid disperse.

105 Preferably, as emulsifying agents, sulphonated wax containing oil or sulphonated waxes and particularly the sulphonated oil-and-wax mixtures or sulphonated liquid

waxes or the sulphonation products of material proportions of liquid waxes derived from marine animals are employed.

The liquid waxes include the "oil" from the "case" of the true sperm whale, *Physeter macrocephalus*, and the oil from the head cavity of the bottlenose whale, *Hyperoodon rostratus* and *Hyperoodon diodon*, both "oils" being, it is believed, described in commerce as "sperm oil". Other oils obtainable commercially, for instance the oil from the blubber of the whales above referred to, contain material proportions of liquid waxes, and the products obtained by the sulphonation of such "oils" are suitable for use.

Highly satisfactory results may be secured in accordance with the invention by using as the emulsifying agent sulphonated sperm oil which may also act as a tempering agent, and by the use of sperm oil as the oily or waxy constituent of the stencil layer or main tempering agent. The invention is, however, not confined to the use of sperm oil in this capacity as many other oils, including for instance mineral oils, are suitable for use in accordance with the invention.

In this connection it may be remarked that the employment of Turkey red oil in association with fatty bodies and gelatinizing organic colloids, such as gelatine, dispersed in water has been proposed in the production of stencil sheets. I have found, however, that sulphonated castor oil and its derivatives, such as Monopol soap, are entirely unsuitable in the circumstances heretofore prescribed for use in accordance with the invention as they are incapable in such circumstances of securing the dispersion of the oily or fatty material throughout the gelatine or the like to produce a product in which the oily-waxy or waxy material is present in a degree of sub-division comparable with that regarded as a characteristic of colloid particles.

The oily-waxy or waxy constituents are present in the stencil layers in accordance with the invention in such proportion that they constitute wholly or mainly the tempering agent for the organic colloid such as gelatine, that is to say, the agent adapted so to modify the properties of the colloid that the structure of the stencil layer may be broken down by the blows of the type when used in forming stencils in a typewriter or by the style when producing a stencil by hand.

The proportion of the tempering agent I have found it convenient to employ may vary between six and ten parts to one of a colloid, such as gelatine. This indication, however, is only given for the purpose of illustrating the proportion I have found it convenient to use in certain atmospheric or climatic conditions.

An opaque pigment, the colour of which will contrast with the ink with which the stencil will be used, for instance a white pigment, may be incorporated in the stencil layer, as indicated in the specification of the co-pending application for Letters Patent No. 645,708 care being taken to select a pigment which does not operate to break down the structure of the coating composition.

The coating of the porous material forming the base of the stencil sheet may be effected in the usual manner by the employment of a trough or roller, the coated sheet being then dried without, however, subjecting it to treatment which would cause the composition constituting the stencil layer to liquefy.

Further, the coated sheet may be formalized or otherwise treated to convert the organic colloid, such as gelatine, present therein into the insoluble or hardened form.

As is well known, gelatines vary considerably in their properties; for instance, some are more acid than others. It is therefore important to select a gelatine, the properties of which are not inimical (in consequence, for example, of the presence of impurities in it) to the formation of a stable colloid when it is brought together with the oily or waxy bodies and the emulsifying agent.

The following particulars are given by way of example to illustrate a suitable method of carrying the invention into effect.

A coating composition is prepared by mixing 150 parts of a 10% aqueous "solution" of gelatine with 25 parts of sulphonated sperm oil and 75 parts of sperm oil and adding 20 parts of a composite white titanium oxide pigment. The composition when uniform and diluted to a suitable viscosity is introduced into the tank of a coating machine of the kind in which the material to be coated is drawn over a roller partly immersed in the coating composition, meanwhile maintaining the composition at a temperature substantially over its gelating temperature, for example, 100° F. to 140° F.

The coated sheets are then allowed to dry, care being taken to avoid liquefying the composition during this operation.

The coated sheets may then be formalized by passing them through a chamber in which an atmosphere containing formaldehyde is maintained.

It is to be understood that the expressions employed herein in attempting to define the scope of the invention may by further research be found inappropriate; they are, however, believed to be sufficient to define the invention in accordance with current conceptions in the realm of physical chemistry.

Further, as used in the claims, the expression "oily body" includes bodies which are in fact waxes or contain material propor-

tions of waxes and "sulphonated wax" and "sulphonated liquid wax" include products obtained by the sulphonation of oils containing material proportions of wax.

5 Having now described my invention, what I claim as new and desire to secure by Letters Patent is:—

1. A stencil sheet for use in duplicating manuscript and typewritten documents, 10 drawings and the like, comprising a stencil layer in the form of a disperse system including a gelatinized organic colloid deposited from an aqueous medium, an oily body as the main tempering agent and a sul- 15 fonated material containing a sulfonated wax adapted to secure the desired degree of dispersion of the oily body in the stencil layer.

2. A stencil sheet for use in duplicating 20 manuscript and typewritten documents, drawings and the like, comprising a stencil layer in the form of a disperse system including a gelatinized organic colloid deposited from an aqueous medium, an oily body 25 as the main tempering agent and a sulfonated wax.

3. A stencil sheet for use in duplicating 30 manuscript and typewritten documents, drawings and the like, comprising a stencil layer in the form of a disperse system including a gelatinized organic colloid deposited from an aqueous medium, an oily body as the main tempering agent and a sulfonated liquid wax.

35 4. The process of forming stencil sheets which comprises applying to a porous support, for instance yoshino paper, an emulsion from which volatile organic solvents

are absent, comprising a gelatinizing organic colloid dispersed in an aqueous medium, 40 an oily body in a proportion considerably in excess of the said colloid, and functioning as the main tempering agent, and a sulphonated wax.

5. The process of forming stencil sheets 45 which comprises applying to a porous support, for instance yoshino paper, an emulsion from which volatile organic solvents are absent, comprising a gelatinizing organic colloid dispersed in an aqueous medium, 50 an oily body in a proportion considerably in excess of the said colloid, and functioning as the main tempering agent, and a sulphonated liquid wax.

6. The process of forming stencil sheets 55 which comprises applying to a porous support, for instance yoshino paper, an emulsion from which volatile organic solvents are absent, comprising a gelatinizing organic colloid dispersed in an aqueous medium, 60 an oily body in a proportion considerably in excess of the said colloid, and functioning as the main tempering agent, and a sulphonated sperm oil.

7. A stencil sheet comprising a base of 65 open porous material coated with a composition comprising a gelatinized organic colloid, an oily material and a liquid sulfonated oil, such composition being substantially free from hygroscopic materials, such 70 stencil sheet being adapted to remain permanently in condition for stencilizing in the dry state.

In testimony whereof I have signed my name to this specification.

ARMAND DE WAELE.